

# United States Patent Office

2,836,508

Patented May 27, 1958

1

2,836,508

## DRYING OIL POLYMER CONTAINING AN ACIDIC PHOSPHORUS COMPOUND

Thomas L. Canniff and Alfred E. Balocca, Wheaton, Ill., assignors to American Can Company, New York, N.Y., a corporation of New Jersey

No Drawing. Application July 9, 1954  
Serial No. 442,428

6 Claims. (Cl. 106—285)

The present invention relates to a novel, economical and effective coating composition. More particularly the present invention pertains to a modified diolefin polymer coating composition for sheet metal, and especially containers fabricated from ferrous metal sheets.

The use of organic coatings on sheet metal as a protection therefor is old and well known. However due to certain special problems in can manufacture, relatively few of the known coating compositions are applicable to can making. The maximum thickness of the coating on metal cans is but a fraction of the usual thickness of the coatings on other metal surfaces. This extremely thin coating must be hard so as to resist marring during abuse in fabrication and handling of the cans; it must be flexible in order to form a continuous adherent film over can parts that have been fabricated by drawing or bending; and it must be substantially impervious to chemical attack. In relation to the last requirement such a variety of products are packed in cans, each presenting its own corrosive problem, that heretofore there has been no single organic coating composition that is effective against the different types of chemical attack. Therefore it is necessary to develop and use a different coating to resist each particular type of corrosion. Obviously such an operation is costly and troublesome.

During recent years this situation has been aggravated by the tremendous increase in the use of organic coatings over tin coatings. Previously most, if not all, metal containers were made from sheet steel having a protective coating of tin on its surfaces. This involved a tremendous consumption of tin in view of the fact that billions of metal containers are manufactured each year. Due to the growing scarcity of tin and the fact that tin has to be imported from foreign countries such as Malaya, Bolivia and the Belgian Congo, a constant effort has been made by the container manufacturing industry to develop substitute coating compositions and methods whereby to conserve tin or obviate its use entirely. In relation to protective coatings for steel plate, one method of tin conservation has been to reduce drastically the weight of tin deposited on sheet steel and provide supplemental protection by the use of organic coatings thereover. Another method has been to eliminate entirely the use of tin coating and obtain corrosion protection solely by the use of organic coatings.

2

After extensive experimentation with many different materials we have discovered that by modifying a particular diolefin polymer with a small amount of an acidic phosphorus compound and thereafter applying this novel composition to the surface of a ferrous metal plate and treating the coated plate we could produce a thin, hard, adherent, flexible, heat-stable film thereon which protects the metal substrate from atmospheric and other chemical corrosion and that this film withstood the severe drawing, bending and shaping operations prevailing in sheet metal container manufacture.

Therefore an object of this invention is to provide a substantially universal organic coating for metal containers.

15 Another object of this invention is to provide a substantially universal organic coating for metal containers that is equivalent in quality and protective value and manufacturing ease to tin coated containers and which is more readily available and less costly than tin.

20 Another object of this invention is to provide a substantially universal organic coating for ferrous metal containers and many other ferrous products that is more economical and in many respects superior to organic coatings presently and heretofore in use.

25 Another object of this invention is to provide a substantially universal, tough and flexible organic coating for all types of fabricated sheet metal products which in the course of manufacture have to undergo severe bending, drawing and shaping operations.

30 Numerous other objects and advantages of the invention will be apparent as it is better understood from the following description which is of a preferred embodiment thereof.

35 The particular polymer discovered as useful in the present invention is a synthetic drying oil. This drying oil is a normally liquid, oily homopolymer of an aliphatic, open chain, conjugated diolefin, particularly butadiene-1,3.

40 Although it has been found that butadiene-1,3 yields an outstanding drying oil, homologues of butadiene having up to 6 carbon atoms such as isoprene, piperylene and 2,3-dimethyl butadiene-1,3 also yield a satisfactory product. These homologues may be substituted for all or 45 part of the butadiene-1,3 or mixtures of these homologues may be used.

50 In the polymerization of the diolefin monomer, boron trifluoride was found to be the most effective polymerization catalyst. The finished polymer has an average molecular weight of about 1600 to 1800 as calculated by the boiling point elevation method, and a relative viscosity of about from 1.15 to 1.25.

55 Relative viscosity ( $N_r$ ) is the value of the fraction:

55 (A) Efflux time of polymer solution

55 (B) Efflux time of solvent used in polymer solution

60 The efflux times are measured in accordance with the procedure of the American Society for Testing Materials

D-445-46T Method B, using as the "oil" mentioned in the procedure, (A) a solution of 350 milligrams of the polymer in 25 cc. of C. P. benzene, and (B) a sample of the C. P. benzene used in making the solution of (A). The determinations are run at 25° C. in a modified Ostwald viscosimeter, series 50.

The above described synthetic drying oil polymer is more fully described in copending application, Serial No. 361,861, filed June 15, 1953, Patent No. 2,777,890.

The above described synthetic drying oil polymer without the addition of the acidic phosphorus compound, while showing promise as an organic coating for metal containers is deficient in that regard in many important factors, e. g. blistering, discoloration, adhesion and especially flexibility. This last deficiency results in the corrosion of container parts fabricated from plate having the unmodified polymer as a coating thereon due to fracture of the coating at points where the substrate metal is subjected to stress or bending.

We have discovered the surprising and unexpected fact that the addition of a small amount of an acidic phosphorus compound to the polymer alleviates these deficiencies yielding a composition having in all respects exceptional properties as a metal container coating. It is believed that this remarkable improvement is due to the acidic phosphorus compound inhibiting oxidative polymerization of the cross-linking type during the curing of the film thereby yielding a less brittle, more adherent, and more flexible film. However, since these theoretical considerations form no part of the present invention, we do not wish to be bound thereby.

Another surprising and unexpected result obtained by the incorporation of an acidic phosphorus compound in a drying oil film according to the present invention is the marked improvement in the heat stability of the film. When the side seam of a can body is bonded by means of molten solder having a temperature of 700° F. or more, a great deal of heat is applied to the inside coating of the body adjacent the side seam. This large amount of heat usually causes severe scorching and discoloration of the coating in the area of the side seam and in some instances causes this portion of the coating to break down and develop holes. We have found that the coating compositions of our invention are remarkably resistant to heat, displaying very little scorching or discoloration and no break-down whatsoever when subjected to the high temperatures of the soldering operation.

The term acidic phosphorus compound used herein designates phosphorus acids, phosphorus acid derivatives having at least one replaceable acidic hydrogen atom and mixtures thereof. Included in the phosphorus acids are ortho-, meta-, hypo-, and pyrophosphoric acid, phosphorous acids, polyphosphoric acid and any phosphorus compound that will yield a phosphoric acid in aqueous solution, e. g. hydrates of orthophosphoric acid, anhydrous phosphoric acid, phosphorus pentoxide, phosphoric oxide, phosphoric anhydride,  $P_2O_5$  and  $P_4O_{10}$ . Of the phosphorus acid derivatives we include: inorganic salts of phosphorus acid such as zinc acid phosphate and ammonium acid phosphate; organic esters of phosphorus acids such as alkyl phosphates, e. g. n-amyl phosphate and dibutyl phosphate; and organic salts of phosphorus acids such as amine phosphates, e. g. mono-(dibutylamine) pyrophosphate, dianiline phosphate and dibenzylamine phosphate. Of the acidic phosphorus compounds disclosed, the unsubstituted phosphorus acids produce superior results and therefore are preferred.

In accordance with the invention the acidic phosphorus compound is dissolved in a suitable solvent. An amount of this solution is slowly added to an already prepared solution of the drying oil polymer so that the resulting product contains a major portion of polymer and a minor portion of acidic phosphorus compound. Based upon

the weight of polymer in the composition, between 0.1% and 8% of acidic phosphorus compound and preferably between 0.50% and 4.0% is incorporated in the composition. These limits are critical since an amount of acidic phosphorus compound less than the minimum limit fails to give the desired result and an amount thereof greater than the upper limit inhibits curing of the film to an excessive degree causing it to be soft and tacky. If the acidic phosphorus compound solution is insoluble in the polymer solution, the addition must be accompanied by vigorous agitation of the mass so that the former is uniformly dispersed throughout the latter yielding a homogeneous product. However, with certain acidic phosphorus compounds, e. g. some organic phosphates, a solvent compatible with the synthetic drying oil solution can be used so that a clear solution of acidic phosphorus compound solution in polymer solution can be obtained. With other acidic phosphorus compounds, it may be advantageous to add them as a solid or in the form of a thick slurry. This may be accomplished by milling the acidic phosphorus compound into the polymer.

The time of mixing or temperature of the ingredients is not critical, varying over a wide range. The only limitation as to time of mixing is that sufficient time be allowed to insure uniform and intimate contact of the ingredients. In general 5 to 15 minutes should be sufficient. As to temperature, it is necessary only that the solutions be liquid, i. e. above their freezing points.

Solvents such as water, lower aliphatic alcohols, normally liquid ketones and combinations thereof can be used as solvents for the acidic phosphorus compounds. Inert organic liquids having a boiling range between 20° C. and 200° C. may be used as solvents for the polymer. Aliphatic hydrocarbons such as solvent naphtha and mineral spirits, e. g. Varsol (boiling range about 150° C. to 200° C.), Solvesso (boiling range about 95° C. to 200° C.), are preferred. Aromatic solvents such as benzene, toluene and xylene may also be used but are not as desirable as the aliphatic solvents due to their toxicity.

In the acidic phosphorus compound modification of the polymer the selection of a proper solvent is not critical depending merely upon the degree of solubilities of the respective ingredients therein.

In the coating operation, the metal sheet may be either spray, dip or roller coated. The procedure generally used in metal container manufacture is the roller coating of flat metal sheets as by an apparatus similar to that disclosed in United States Patent 1,848,836, issued to C. Wagner et al. on March 8, 1932. The resin coating is then cured at an elevated temperature usually by means of a device similar to that shown and described in United States Patent 1,293,261, issued to C. Wagner et al. on February 4, 1919.

In applying the coating composition of the present invention by the roller coating process, the liquid coating composition should have a viscosity of between 90 and 315 centistokes and preferably between 175 and 250 centistokes and a solids content of not less than 20 percent by weight of the total liquid composition. In actual operation the solids content is in the range of 40 percent to 60 percent by weight of the total. To effect a cure, the resin coating is baked at a temperature of from 375° F. to 420° F. for 8 to 15 minutes. The cured film is approximately from  $2.5 \times 10^{-4}$  to  $8.5 \times 10^{-4}$  cm. thick over the metal substrate which corresponds to a weight of approximately 2 mg. per square inch to 5 mg. per square inch respectively of metal plate surface.

The following tabulation will serve to illustrate specific embodiments of the present invention but are in no way intended as limitations thereon. In each of the following examples, the major constituent of the composition is a butadiene polymer as described hereinbefore:

5  
EXAMPLES

## 6

| No.    | Modifier                                                                       | Percent Modifier added <sup>1</sup> | Solvent                 | Percent Solids of Composition <sup>2</sup> | Viscosity in Centi-strokes |
|--------|--------------------------------------------------------------------------------|-------------------------------------|-------------------------|--------------------------------------------|----------------------------|
| 1..... | o-phosphoric acid                                                              | 1, 2, 4                             | Butanol-Toluene         | 45                                         | 210                        |
| 2..... | phosphorous acid                                                               | 1, 2, 4<br>6, 7, 8                  | do                      | 45                                         | 210                        |
| 3..... | polyphosphoric acid                                                            | 1, 2, 4                             | do                      | 45                                         | 210                        |
| 4..... | dibutyl-phosphate                                                              | 1, 2, 4                             | do                      | 45                                         | 210                        |
| 5..... | mono-(dibutylamine)-pyrophosphate                                              | 1, 2, 4                             | do                      | 45                                         | 210                        |
| 6..... | zinc dihydrogen phosphate Zn<br>(H <sub>2</sub> PO <sub>4</sub> ) <sub>2</sub> | 1, 2, 4                             | Mineral Spirits         | 45                                         | 210                        |
| 7..... | dianiline phosphate                                                            | 1, 2, 4                             | Butanol-Mineral Spirits | 45                                         | 210                        |

<sup>1</sup> Each number represents a different composition having that percent by weight of polymer of the particular acidic phosphorus compound designated.

<sup>2</sup> This represents percent by weight of total composition.

Small amounts of other substances may be incorporated into the novel composition of the present invention depending upon the result desired. Included in these are pigments such as aluminum and titanium oxide; waxes as internal lubricants; inhibitors; and vegetable drying oils. A small amount of rubber, natural or synthetic, may be added to improve the elasticity of the coating.

The data tabulated below shows the superiority of the coating of the present invention over all the other coatings rated on the products shown, thereby illustrating its value as a single replacement for the different coatings generally in use. Table I compares the properties of a coating composition of the present invention, i. e. polybutadiene drying oil modified with 1.0% by weight of drying oil of o-phosphoric acid, to those of the unmodified drying oil and to those of commercial can coatings used in packing corn and pumpkin. The metal substrates used in these tests were CMQ plate (Can Maker's Quality uncoated steel sheet), tin plate having low weight of tin coating per base box of steel (.25 lb.) and tin plate having a high weight of tin coating per base box of steel (1.25 lb.). These coated sheets were then fabricated into container parts and contacted with the products designated below, each coating receiving identical treatment in its contact with the respective products. The coated metal can part was then removed from the product and evaluated, the results of which are shown in the table below. In the numerical ratings given in Table I, zero is perfect ranging upward therefrom to unsatisfactory.

It is thought that the invention and many of its attendant advantages will be understood from the foregoing description, and it will be apparent that various changes may be made in the matter of the ingredients, their identity and their proportions without departing from the spirit and scope of the invention or sacrificing all of its material advantages, the form hereinbefore described being merely a preferred embodiment thereof.

We claim:

- 30 1. A coating composition comprising an oily liquid conjugated diolefin polymer synthetic drying oil formed using a boron trifluoride polymerization catalyst, and from 0.5% to 4.0% by weight of said drying oil polymer of a phosphorus compound having at least one replaceable acidic hydrogen atom, said diolefin containing 4 to 6 carbon atoms, and said polymer having a molecular weight of about from 1600 to 1800 and a relative viscosity of about from 1.15 to 1.25.
- 35 2. A coating composition comprising an oily liquid butadiene-1,3 polymer synthetic drying oil formed using a boron trifluoride polymerization catalyst, and from 0.5% to 4.0% by weight of said drying oil polymer of a phosphorus compound having at least one replaceable acidic hydrogen atom, said polymer having a molecular weight of about from 1600 to 1800 and a relative viscosity of about from 1.15 to 1.25.
- 40 3. A coating composition comprising an oily liquid butadiene-1,3 polymer synthetic drying oil formed using a boron trifluoride polymerization catalyst, and from 0.5% to 4.0% by weight of said drying oil polymer of a phosphorus compound having at least one replaceable acidic hydrogen atom, said polymer having a molecular weight of about from 1600 to 1800 and a relative viscosity of about from 1.15 to 1.25.
- 45 3. A coating composition comprising an oily liquid butadiene-1,3 polymer synthetic drying oil formed using a boron trifluoride polymerization catalyst, and from 0.5% to 4.0% by weight of said drying oil polymer of

Table I

| Coating                     | Metal Substrate | Pumpkin          |                  | Corn             |                  | Pork             |                  |
|-----------------------------|-----------------|------------------|------------------|------------------|------------------|------------------|------------------|
|                             |                 | Process Resist.  | Flexib.          | Process Resist.  | Flexib.          | Process Resist.  | Flexib.          |
| Unmodified polymer.....     | CMQ.....        | 8.9              | 15.3             | 4.6              | 11.6             | 14.5             | 19.4             |
| Do.....                     | .25 lb.....     | 4.7              | 11.7             | 2.6              | 5.7              | 7.0              | 15.0             |
| Do.....                     | 1.25 lb.....    | 3.3              | 9.0              | 2.0              | 5.6              | 11.3             | 11.3             |
| Comm'l corn coating.....    | CMQ.....        | ( <sup>1</sup> ) | ( <sup>1</sup> ) | ( <sup>1</sup> ) | ( <sup>1</sup> ) | ( <sup>1</sup> ) | ( <sup>1</sup> ) |
| Do.....                     | .25 lb.....     | 5.3              | 6.0              | 6.3              | 5.6              | 19.6             | 10.0             |
| Do.....                     | 1.25 lb.....    | 8.3              | 6.3              | 7.3              | 6.4              | 24.7             | 9.0              |
| Comm'l pumpkin coating..... | CMQ.....        | ( <sup>1</sup> ) | ( <sup>1</sup> ) | ( <sup>1</sup> ) | ( <sup>1</sup> ) | ( <sup>1</sup> ) | ( <sup>1</sup> ) |
| Do.....                     | .25 lb.....     | 5.0              | 6.9              | ( <sup>1</sup> ) | ( <sup>1</sup> ) | ( <sup>1</sup> ) | ( <sup>1</sup> ) |
| Do.....                     | 1.25 lb.....    | 3.0              | 6.0              | ( <sup>1</sup> ) | ( <sup>1</sup> ) | ( <sup>1</sup> ) | ( <sup>1</sup> ) |
| modified polymer.....       | CMQ.....        | 5.1              | 10.4             | 6.3              | 7.7              | 6.0              | 10.3             |
| Do.....                     | .25 lb.....     | 3.8              | 6.0              | 3.3              | 4.3              | 8.3              | 8.0              |
| Do.....                     | 1.25 lb.....    | 2.2              | 5.0              | .9               | 7.0              | 9.9              | 12.4             |

<sup>1</sup> Complete failure.

While the novel composition of the present invention has been described specifically as a metal can coating, it has utility of much greater scope. This polymer forms an excellent protective coating on all metal substrates, particularly ferrous metal substrates, where a tough, flexible, adherent, corrosion resistant, heat-stable, continuous film is desired.

70 a member of the group consisting of an unsubstituted acid of phosphorus, an acid phosphate having at least one replaceable acidic hydrogen atom, an acid phosphite having at least one replaceable acidic hydrogen atom and mixtures thereof, said polymer having a molecular weight of about from 1600 to 1800 and the relative viscosity of about from 1.15 to 1.25.

4. The composition of claim 3 in which the unsubstituted acid of phosphorus is ortho phosphoric acid.
5. The composition of claim 3 in which the unsubstituted acid of phosphorus is phosphorous acid.
6. The composition of claim 3 in which the unsubstituted acid of phosphorus is polyphosphoric acid. 5

## References Cited in the file of this patent

## UNITED STATES PATENTS

|           |              |                |
|-----------|--------------|----------------|
| 2,240,081 | Thomas       | Apr. 29, 1941  |
| 2,587,477 | Hunter       | Feb. 26, 1952  |
| 2,641,551 | Smith et al. | June 9, 1953   |
| 2,652,342 | Gleason      | Sept. 15, 1953 |
| 2,666,034 | Bishop       | Jan. 12, 1954  |